

# UNITED STATES PATENT OFFICE.

CALVIN VOS, OF NEW YORK, N. Y.

## ALLOY.

1,382,146.

Specification of Letters Patent. Patented June 21, 1921.

No Drawing.

Application filed April 10, 1920. Serial No. 372,954.

To all whom it may concern:

Be it known that I, CALVIN Vos, a citizen of the United States, residing at New York, in the county of New York and State 5 of New York, have invented certain new and useful Improvements in Alloys, of which the following is a specification.

This invention relates to an improvement in alloys.

10 The main object of the invention is to produce an alloy to be used as an agent in the manufacture of steel for any purpose and for making iron and steel castings, which product possesses unusual tensile 15 strength and toughness, said alloy possessing degasifying and deoxidizing properties which render the same of especial value in the manufacture of a flawless product in which such qualities and characteristics are 20 particularly essential and of great value.

With the above named object in view, this invention comprises an alloy including the composition of metals hereinafter described and set forth, and particularly 25 pointed out in the claims.

My improved alloy consists of aluminum within the limits of from 90 to 95 per cent.; magnesium within the limits of from 2 to 10 per cent.; sodium fluorid within the limits 30 of from 0.01 to 5 per cent.; uranium in the oxid state within the limits of from 0.01 to 6 per cent., and ferrosilicon within the limits of from 0.2 to 3 per cent.

In the manufacture of the alloy, my 35 method of procedure is as follows:

I first melt the aluminum in a suitable container, then apply heat to raise the temperature of the aluminum sufficiently to reduce it to a molten mass, then I introduce 40 the sodium fluorid, ferrosilicon and uranium oxid, constantly stirring and agitating the whole mass gently.

After the aluminum, sodium fluorid, uranium oxid and ferro-silicon shall have been 45 thoroughly melted and mixed together, I then add the magnesium, so that when the metals herein referred to are thoroughly melted and mixed by constant gentle stirring, the alloy produced is admirably adapted for use in degasifying and deoxidizing steel and the ferrous groups of metals, thereby increasing the density and eliminating the tendency of formation of flaws in the castings obtained from said metals.

It will be understood that when all of the 55 metals have been properly mixed and reduced to a molten mass, the constant gentle stirring action will cause such gases as may be contained in the molten metal to escape therefrom, thereby insuring a more dense 60 and homogeneous product.

By means of the ingredients and my method hereinbefore referred to, an improved alloy is obtained which is possessed of unusual tensile strength and density, and 65 which is especially desirable in the manufacture of steel and iron and steel castings where it is important that the product shall possess flawless qualities and the maximum strength.

It will be evident that the compounds mentioned do not remain in the finished alloy in the same proportions hereinbefore referred to, since the sodium fluorid serving as a fluxing agent will have substantially disappeared, also some of the ferro-silicon and a part of the oxygen of the uranium oxid, thereby forming a finished alloy composed of aluminum of approximately from 90 to 95 per cent.; magnesium 80 approximately from 1.5 to 9.15 per cent.; uranium approximately from .005 to 2.75 per cent.; ferro-silicon approximately from .05 to 1.25 per cent., and iron approximately from .1 to 1.80 per cent.

Having fully described my invention, what I claim and desire to secure by Letters Patent is:

1. An alloy possessing degasifying and deoxidizing properties used in the production of steel and iron and steel castings having unusual strength and density, composed of a major portion of aluminum, a reduced portion of magnesium, and a minor quantity of uranium, ferro-silicon and iron.

2. An alloy having degasifying and deoxidizing properties for eliminating all oxides and gases from the steel, composed of aluminum, magnesium, uranium, ferro-silicon and iron, the aluminum being approximately from 90 to 95 per cent.; the magnesium approximately from 1.5 to 9.5 per cent.; uranium approximately from .005 to 2.75 per cent.; ferro-silicon approximately from .05 to 1.25 per cent., and iron approximately from .1 to 1.80 per cent.

CALVIN VOS.